

## UNITED STATES PATENT OFFICE

2,512,674

## PRODUCTION OF CASEIN YARN

Robert F. Peterson, Philadelphia, Pa., assignor to  
the United States of America as represented by  
the Secretary of Agriculture

No Drawing. Application June 13, 1947,  
Serial No. 754,583

2 Claims. (Cl. 18—54)

(Granted under the act of March 3, 1883, as  
amended April 30, 1928; 370 O. G. 757)

1

This application is made under the act of March 3, 1883, as amended by the act of April 30, 1928, and the invention herein described, if patented, may be manufactured and used by or for the Government of the United States of America for governmental purposes without the payment to me of any royalty thereon.

This invention relates to casein yarn, and has among its objects a process of producing yarn in a simple and expeditious manner from casein fibers having enhanced tensile strength, softness and flexibility.

It is known that casein fiber may be spun from an alkaline solution of casein into a precipitating bath of about 10% sulfuric acid and 14% sodium sulfate, and the fiber then stretched while passing through a heated hardening bath containing about 10% aluminum sulfate, 10% sodium sulfate and 5% formaldehyde. Analyses of the fiber at this stage show that it contains only 0.2 to 0.5% combined formaldehyde not removed by washing. In order to be dimensionally stable in the unrelaxed state, the fiber must contain about 1.5% reacted formaldehyde. The time to attain this amount might require as long as 30 minutes of processing under tension. The rate of the formaldehyde reaction may be increased by raising the temperature, but this rate passes through a maximum in most baths so that higher temperatures remove formaldehyde and reverse the hardening reaction.

In order to produce dimensionally stable fiber under these conditions, it may be wound under tension onto a bobbin to prevent shrinkage and loss of tensile strength, and the bobbin and fiber placed in the formaldehyde and salt solution for the required time. In this procedure, however, enough shrinkage occurs to felt the inner layers of fiber on the bobbin together so that the bobbin can be unwound only partially, and much of the fiber is wasted.

To construct the fiber spinning machine so that the requisite formaldehyde needed to stabilize the fiber is reacted without winding the fiber requires a considerably increased floor space for each unit.

Some improvement may be obtained by substituting an acetic acid precipitating bath for the sulfuric acid bath, using 5 to 10% acetic acid and saturated sodium sulfate solution. If, now, the fiber from this bath is wound on a bobbin and placed in the formaldehyde and salt solution in the manner mentioned above, all the finished fiber will unwind from the bobbin, but the individual fibers within the tow will be

2

partially fused, and the yarn produced from them cannot be knit as it lacks flexibility. The only advantage attaching to the use of such acetic acid precipitating bath is that the shrinkage of the fibers after the removal of tension will be reduced compared to fibers from the sulfuric acid bath.

In general, according to the present invention, threads of an alkaline casein solution are extruded or spun into an organic acid precipitating bath in the usual manner to precipitate the casein into fibers, and the precipitated fibers then treated under tension in a heated fixing solution containing a metal salt and formaldehyde for a short interval to give partially hardened fibers having about from 0.2 to 0.5% combined formaldehyde. The fibers are then immediately immersed in a concentrated buffer solution having a pH of 6 to 8. This stabilizes the fibers and further strengthens and hardens them so that they can immediately thereafter be spun into yarn under tension, even using the so-called "pot" centrifuge method, which is drastic in its tendency to unite the fibers, without the fibers being stuck together either within the yarn by the twisting as they enter the funnel of the centrifuge or between the layers of yarn in the cake.

The following example exhibits the process in greater detail.

An aqueous solution containing 20% casein and 0.4% NaOH was spun at room temperature into a precipitating bath containing 5% acetic acid, 20% sodium sulfate and 5% glucose. The spinnerette used contained 250 holes each of .003 inch diameter, the gear pump delivered 5.4 ml. of casein solution per minute, and the extruded threads traveled through the precipitating bath for 20 inches. The draw-off wheel operated at a surface speed of 9 meters a minute, and the tow passed next to a set of conical grooved rollers spaced a meter apart, the lower of which dipped into a heated aqueous fixing solution containing 10% aluminum sulfate, 10% sodium sulfate and 5% formaldehyde, and held at 60° C. The tow made 5 loops in passing from the inner 4-inch diameter grooves to the outer 8-inch diameter grooves, and thus was under sufficient tension to receive a 100% stretch. An additional 83% stretch was imposed on the tow as it left the conical rolls by running the next set of rolls at a higher speed.

On this next set of cylindrical rolls, the fiber was stabilized with the bath buffered to a pH of 6,

3 by immersing the lower roller in a 30% aqueous sodium acetate solution.

The fiber was then immediately spun into yarn by being dropped into the funnel of a centrifuge unit similar to those used in spinning viscose rayon by the "pot" method. The cake of yarn was removed every 2 to 3 hours, washed to remove soluble salts, and dried in a circulating air dryer.

The resulting yarn was about 400 denier, and had a tenacity of 1 gram per denier dry and one-half gram per denier wet. The breaking elongation was about 50% either with the fiber dry or wet. The yarn thus produced knits well on a knitting machine and the finished fabrics have a soft, silky feel, are a lustrous white, and can be dyed easily.

In the above example, other lower fatty acids or hydroxy fatty acids, such as formic acid or lactic acid, may be substituted for the acetic acid in making up the precipitating bath, and other metal salts such as salts of chromium, zirconium and beryllium may be substituted for the aluminum sulfate in the heated salt bath.

It is essential, however, that the pH of the concentrated buffer solution be controlled to the limits indicated, and that the treatment be given immediately following the treatment in the hot salt bath (that is, prior to spinning the fiber in the yarn), for if the fibers be spun into yarn or wound without the treatment, they will be stuck together in the yarn, and immersion in the buffer solution thereafter is of no avail.

The resulting yarn is eminently suited for knitting. It is soft and flexible, and the knitted fabrics made from it have the sroop characteristic of silk. This action of the concentrated buffer is unexpected, since even fibers washed at pH 5 where hydration should be at a minimum do not exhibit this softness. The softness is increased tenfold by washing at pH 6 instead. No additional treatment with formaldehyde solutions is required after the fiber is wound.

The improvement produced by this invention in degree of flexibility of the finished yarn may be given a numerical value by using the 0.5 inch-pound model of the Olsen-Tour-Marshall stiffness tester. Several fibers must be mounted in parallel and the lowest capacity range of the machine (.005 inch-pound) is used, with a  $\frac{1}{8}$  inch span. Data follow on yarn from several cakes spun on the machine which differ only in the nature of the treatment before entering the pot. The

5 "stiffness" of the last column was measured in each case at 45 degrees angle of bending.

| No. of yarn sample | Treatment                 | No. filaments/denier | "Stiffness" in inch-lbs. |
|--------------------|---------------------------|----------------------|--------------------------|
| 1-----             | No wash bath-----         | 250/400              | $0.230 \times 10^{-2}$   |
| 2-----             | Wash at pH 5-----         | 250/400              | $0.180 \times 10^{-2}$   |
| 3-----             | Wash at pH 6-----         | 250/400              | $0.016 \times 10^{-2}$   |
| 10                 | Commercial viscose rayon. | 100/300              | $0.016 \times 10^{-2}$   |

15 The pH 6 wash softens the fiber until the yarn is comparable to a 300 denier viscose yarn which has been oiled, ready for knitting. The casein yarns measured were not oiled. If the stiffer yarns are oiled and subjected to considerable mechanical working, the yarn adhesions can be partially broken up, but the softness still does not approach that of the fiber washed at pH 6. In addition, many of the filaments of such stiffer yarn 20 are broken, and this provides an added source of trouble during knitting. Also, the knitted fabrics from these yarns are harsh and stiff.

Having thus described the invention, what is claimed is:

25 1. A process of producing casein yarn comprising extruding threads of an alkaline solution of casein into an organic acid precipitating bath to precipitate the casein into fibers, treating the precipitated fibers under tension with a heated fixing solution containing a metal salt and formaldehyde to give partially hardened fibers, then immediately immersing the partially hardened fibers in a concentrated buffer solution having a pH of 6 to 8 to stabilize the fibers and further to harden and strengthen them, and then immediately spinning the fibers into yarn while maintaining them under tension.

30 2. The process of claim 1, wherein the buffer solution consists essentially of aqueous sodium acetate.

40 ROBERT F. PETERSON.

#### REFERENCES CITED

45 The following references are of record in the file of this patent:

#### UNITED STATES PATENTS

| Number       | Name         | Date          |
|--------------|--------------|---------------|
| 50 2,211,961 | Meigs        | Aug. 20, 1940 |
| 2,342,994    | Atwood       | Feb. 29, 1944 |
| 2,409,475    | Cline        | Oct. 15, 1946 |
| 2,429,214    | Biehn et al. | Oct. 21, 1947 |